

[72] Inventors **Grant M. Haist;  
Wilbert J. Humphlett; James R. King, all of  
Rochester, N.Y.**  
[21] Appl. No. **764,298**  
[22] Filed **Oct. 1, 1968**  
[45] Patented **Nov. 16, 1971**  
[73] Assignee **Eastman Kodak Company  
Rochester, N.Y.**

[56] **References Cited**  
**UNITED STATES PATENTS**  
3,152,904 10/1964 Sorensen et al..... 96/76  
3,279,920 10/1966 Theodorou..... 96/64 X  
*Primary Examiner*—William D. Martin  
*Assistant Examiner*—Theodore G. Davis  
*Attorneys*—William H. J. Kline, Bernard D. Wiese and Gerald  
E. Battist

[54] **PHOTOSENSITIVE COMPOSITIONS COMPRISING  
SILVER COMPLEXES OF 3-SUBSTITUTED-4-  
THIAZOLINE-2-THIONES AND PHOTOSENSITIVE  
ELEMENTS COMPRISING SUCH COMPOSITIONS**  
23 Claims, No Drawings

[52] U.S. Cl..... 96/94 R,  
96/88  
[51] Int. Cl..... G03c 1/02  
[50] Field of Search..... 96/94, 88,  
65, 64, 114.6, 50; 117/34

**ABSTRACT:** Complex silver salts, formed by silver ion with a 3-substituted-4-thiazoline-2-thione which has an active hydrogen in the group substituted at the 3-position, are found to be photosensitive, i.e., capable of forming photographic images by photoexposure and development, useful for making photographic films, plates and the like.

PHOTOSENSITIVE COMPOSITIONS COMPRISING  
SILVER COMPLEXES OF 3-SUBSTITUTED-4-  
THIAZOLINE-2-THIONES AND PHOTOSENSITIVE  
ELEMENTS COMPRISING SUCH COMPOSITIONS

This invention relates to photography and particularly to novel photosensitive silver compositions and to photographic elements comprising such compositions.

Photosensitive silver halides have been the basis of silver photography for many years. By photoexposure, the silver halides are made to be differentially reducible by photographic developers. Silver halides, as conventionally used in silver halide photographic emulsions, are practically insoluble in water and in conventional photographic developer solutions; it is necessary after exposure and development of a photograph made with photographic silver halide emulsions to stabilize the photography by removing undeveloped silver halide by means of a silver halide solvent.

Among the objects of the present invention are to provide novel photosensitive compositions and to provide photographic elements comprising such compositions, as described more particularly herein. In preferred embodiments, fixing by means of a silver halide solvent is not necessary.

An essential photosensitive image forming component of a photographic composition according to the present invention is a complex formed by silver ion in solution with a 3-substituted-4-thiazoline-2-thione derivative having the formula;



wherein R<sub>1</sub> is an aliphatic organic radical having a terminal acidic hydrogen atom bonded to an oxygen atom (e.g., carboxyalkyl, sulfoalkyl, hydroxyalkyl, and the like) preferably containing one to 12 carbon atoms, and the salts thereof; and each of R<sub>2</sub> and R<sub>3</sub> represents a member selected from the group consisting of hydrogen and organic radicals. Some especially preferred specific compounds corresponding to the above formula include

1. 3-Carboxymethyl-4-methyl-4-thiazoline-2-thione;
2. 3-(2-Carboxyethyl)-4-methyl-4-thiazoline-2-thione;
3. 3-(1,2-Dicarboxyethyl)-4-methyl-4-thiazoline-2-thione;
4. 4-methyl-3-(2-sulfoethyl)-4-thiazoline-2-thione potassium salt;
5. 3-(1-carboxyethyl)-4-methyl-4-thiazoline-2-thione
6. 3-(1-Carboxy-3-methylthiopropyl)-4-methyl-4-thiazoline-2-thione;
7. 3-(2-Carboxyethyl)-4-hydroxymethyl-4-thiazoline-2-thione;
8. 4-Carboxy-3-(1-carboxyethyl)-4-thiazoline-2-thione; and
9. 3-(2-Hydroxyethyl)-4-methyl-4-thiazoline-2-thione.

See *J. Org. Chem.*, 29, 2146 (1964); *J. Chem. Soc.*, 1955, 2990.

Synthesis of 4-thiazoline-2-thiones bearing a carboxy group in the 3-position has been described in *Berichte*, 56, 289 (1923); *Compt. Rendus*, 22, 211 (1938), C.A. 32, 6246<sup>3</sup> (1938); *Journ. Am. Chem. Soc.*, 72, 1879 (1950). These syntheses involve treating a dithiocarbamic acid derived from an amino acid and carbon disulfide with an  $\alpha$ -halogenated

ketone. We have slightly modified the earlier procedure by employing methanol instead of water as solvent and by using two equivalents of amino acid and carbon disulfide per equivalent of  $\alpha$ -halo ketones. In some instances, depending on reaction conditions, an intermediate reaction product, either a 4-hydroxythiazolidine-2-thione or a dithiocarbamate is obtained which can then be dehydrated or cyclodehydrated to the 3-substituted-4-thiazoline thione. We have prepared a variety of 3-substituted-4-thiazoline-2-thiones using amino acids such as glycine; DL- or  $\beta$ -alanine; 4-aminobutyric acid; DL-aspartic acid; taurine; DL-methionine; 6aminohexanoic acid and m-aminobenzoic acid and employing such  $\alpha$ -halo ketones as chloroacetone; phenacyl bromide; 3-chloro-2-butanone; ethyl bromopyruvate; ethyl 2- and 4chloroacetates; 1-acetoxy-3-chloro-2-propanone; 1-butysulfonyl- 3-bromo- 2-propanone and 3-chloro-2,4-pentanedione.

The following syntheses typify preferred procedures for preparing certain 3-substituted-4-thiazoline-2-thiones:

A. 4Acetoxymethyl-3-(2carboxyethyl)-4-thiazoline-2-thione

A mixture of 55.2 grams (0.62 mole) of D,L-alanine and 36.8 grams (0.56 mole) of potassium hydroxide in 150 milliliters of methanol is made with warming and stirring. The small amount of D,L-alanine in excess fails to dissolve. To the stirred mixture cooled in an ice bath is added 34 milliliters (0.56 mole) of carbon disulfide over 20 minutes, forming a gummy, white solid. After the cooled mixture is stirred for one hour, a solution of 42 grams (0.28 mole) of 1-acetoxy-3-chloro-2-propanone in an equal volume of methanol is added, with cooling and stirring, over 20 minutes. The reaction mixture is stirred for 1 hour, with cooling. The reactions are exothermic. Sufficient water, about 200 milliliters, to form a solution is added, and the solution is stirred 15 minutes longer. Methanol is removed in vacuo, leaving a yellow solution. Acidification with excess concentrated hydrochloric acid causes an oil to separate which solidifies on standing overnight. Filtration yields 66 grams of crude product, m.p. 144°. Pure product is obtained after two recrystallizations, amounting to 46 grams of light tan needles.

B. 3-(2-Carboxyethyl)-4-phenyl-4-thiazoline-2-thione

A solution of 10 grams (0.035 mole) of 3-(2carboxyethyl)-4-hydroxy-4-phenylthiazolidine-2-thione in 50 milliliters of glacial acetic acid is refluxed for 0.5 hour. On cooling, crystals form as prisms. Water (100 milliliters) is added, and the crystals are collected, giving 7 grams of the thiazoline, m.p. 134°-136°. A second crop gives 2.5 grams.

C. 3-(2-Hydroxyethyl)-4-methyl-4-thiazoline-2-thione

A solution of 61 grams (1 mole) of 2-aminoethanol and 98.1 grams (1 mole) of potassium acetate is made in 600 milliliters of methanol with warming and stirring. To the stirred solution cooled in an icebath is added 60.3 milliliters (1 mole) of carbon disulfide over 20 minutes. Continued stirring for 2½ hours results in the formation of a white precipitate. A solution of 40 milliliters (0.5 mole) of chloroacetone in an equal volume of methanol is added over 20 minutes to the cooled, stirred mixture and then stirring is continued for 1 hour. Sufficient water is added to form a solution, and methanol is removed in vacuo leaving an oil, which resists crystallization.

The oil is collected by extraction with ether. The combined ether phases are extracted with water and dried over anhydrous sodium sulfate. Ether is distilled off and the final traces of solvent removed in vacuo. The resultant oil readily crystallizes yielding 56 grams of product, m.p. 65°. Recrystallization from water gives product of unchanged melting point.

Table I describes other 3-substituted-4-thiazoline-2-thiones derived from amino acids by such procedures:

TABLE I  
4-thiazoline-2-thiones derived from amino acids

| $R_1$                                                     | $R_2$                                        | $R_3$                             | Formula                                                              | M.P.,<br>$^{\circ}\text{C.}^{\text{(a)}}$ | Yield,<br>percent |
|-----------------------------------------------------------|----------------------------------------------|-----------------------------------|----------------------------------------------------------------------|-------------------------------------------|-------------------|
| $\text{CH}_2\text{CO}_2\text{H}$                          | $\text{CH}_2\text{CO}_2\text{C}_2\text{H}_5$ | H                                 | $\text{C}_9\text{H}_{11}\text{NO}_4\text{S}_2$                       | 142-143                                   | 62                |
| $\text{CH}_2\text{CO}_2\text{H}$                          | $\text{CH}_2\text{CO}_2\text{H}$             | H                                 | $\text{C}_7\text{H}_7\text{NO}_4\text{S}_2$                          | 175-176                                   | 100               |
| $\text{CH}_2\text{CO}_2\text{H}$                          | $\text{CH}_2\text{OCOCH}_3$                  | H                                 | $\text{C}_8\text{H}_9\text{NO}_4\text{S}_2$                          | 162-163                                   | 44                |
| $\text{CH}_2\text{CO}_2\text{H}$                          | $\text{CH}_3$                                | $\text{CO}_2\text{C}_2\text{H}_5$ | $\text{C}_8\text{H}_{11}\text{NO}_4\text{S}_2$                       | 159-160                                   | 83                |
| $\text{CH}_2\text{CO}_2\text{H}$                          | $\text{CH}_3$                                | $\text{CO}_2\text{H}$             | $\text{C}_7\text{H}_7\text{NO}_4\text{S}_2$                          | 224-225                                   | 100               |
| $\text{CH}_2\text{CO}_2\text{H}$                          | $\text{CH}_3$                                | $\text{COCH}_3$                   | $\text{C}_7\text{H}_9\text{NO}_4\text{S}_2$                          | 184-185                                   | 83                |
| $(\text{CH}_2)_2\text{CO}_2\text{H}$                      | H                                            | H                                 | $\text{C}_7\text{H}_7\text{NO}_4\text{S}_2 \cdot \text{H}_2\text{O}$ | 58-60                                     | 71                |
| $(\text{CH}_2)_2\text{CO}_2\text{H}$                      | $\text{CH}_3$                                | H                                 | $\text{C}_7\text{H}_7\text{NO}_4\text{S}_2$                          | 132-134                                   | 95                |
| $(\text{CH}_2)_2\text{CO}_2\text{H}$                      | $\text{CH}_2\text{OCOCH}_3$                  | H                                 | $\text{C}_9\text{H}_{11}\text{NO}_4\text{S}_2$                       | 153                                       | 85                |
| $(\text{CH}_2)_2\text{CO}_2\text{H}$                      | $\text{CH}_2\text{OH}$                       | H                                 | $\text{C}_7\text{H}_7\text{NO}_4\text{S}_2$                          | 141                                       | 84                |
| $(\text{CH}_2)_2\text{CO}_2\text{H}$                      | $\text{CH}_2\text{SO}_2\text{C}_4\text{H}_9$ | H                                 | $\text{C}_{11}\text{H}_{17}\text{NO}_4\text{S}_2$                    | 137-138                                   | 74                |
| $(\text{CH}_2)_2\text{CO}_2\text{H}$                      | $\text{C}_6\text{H}_5$                       | H                                 | $\text{C}_{12}\text{H}_{11}\text{NO}_4\text{S}_2$                    | <sup>b</sup> 136-137                      | 100               |
| $(\text{CH}_2)_2\text{CO}_2\text{H}$                      | $\text{CH}_3$                                | $\text{COCH}_3$                   | $\text{C}_7\text{H}_7\text{NO}_4\text{S}_2$                          | 142-143                                   | 92                |
| $(\text{CH}_2)_2\text{CO}_2\text{H}$                      | $\text{CH}_3$                                | $\text{CO}_2\text{C}_2\text{H}_5$ | $\text{C}_{10}\text{H}_{13}\text{NO}_4\text{S}_2$                    | 145-146                                   | 48                |
| $(\text{CH}_2)_2\text{CO}_2\text{H}$                      | $\text{CH}_3$                                | $\text{CO}_2\text{H}$             | $\text{C}_7\text{H}_7\text{NO}_4\text{S}_2$                          | 206-207                                   | 83                |
| $\text{CH}(\text{CH}_3)\text{CO}_2\text{H}$               | H                                            | H                                 | $\text{C}_7\text{H}_7\text{NO}_4\text{S}_2$                          | 146-148                                   | 38                |
| $\text{CH}(\text{CH}_3)\text{CO}_2\text{H}$               | $\text{CO}_2\text{C}_2\text{H}_5$            | H                                 | $\text{C}_8\text{H}_9\text{NO}_4\text{S}_2$                          | 104                                       | 73                |
| $\text{CH}(\text{CH}_3)\text{CO}_2\text{H}$               | $\text{CO}_2\text{H}$                        | H                                 | $\text{C}_7\text{H}_7\text{NO}_4\text{S}_2$                          | 212                                       | 88                |
| $\text{CH}(\text{CH}_3)\text{CO}_2\text{H}$               | $\text{CH}_2\text{CO}_2\text{C}_2\text{H}_5$ | H                                 | $\text{C}_{10}\text{H}_{11}\text{NO}_4\text{S}_2$                    | 60-61                                     | 42                |
| $\text{CH}(\text{CH}_3)\text{CO}_2\text{H}$               | $\text{CH}_2\text{CO}_2\text{K}$             | H                                 | $\text{C}_7\text{H}_7\text{KNO}_4\text{S}_2$                         | 232                                       | 56                |
| $\text{CH}(\text{CH}_3)\text{CO}_2\text{H}$               | $\text{CH}_3$                                | $\text{COCH}_3$                   | $\text{C}_7\text{H}_7\text{NO}_4\text{S}_2$                          | 136-137                                   | 91                |
| $(\text{CH}_2)_3\text{CO}_2\text{H}$                      | $\text{CH}_2\text{CO}_2\text{C}_2\text{H}_5$ | H                                 | $\text{C}_1\text{H}_{11}\text{NO}_4\text{S}_2$                       | 100-101                                   | 79                |
| $(\text{CH}_2)_3\text{CO}_2\text{H}$                      | $\text{CH}_2\text{CO}_2\text{H}$             | H                                 | $\text{C}_7\text{H}_7\text{NO}_4\text{S}_2$                          | 147-148                                   | 100               |
| $(\text{CH}_2)_3\text{CO}_2\text{H}$                      | $\text{CH}_2\text{SO}_2\text{C}_4\text{H}_9$ | H                                 | $\text{C}_4\text{H}_{10}\text{NO}_4\text{S}_2$                       | 145-146                                   | 60                |
| $(\text{CH}_2)_3\text{CO}_2\text{H}$                      | $\text{C}_6\text{H}_5$                       | H                                 | $\text{C}_{13}\text{H}_{13}\text{NO}_4\text{S}_2$                    | 137-138                                   | 52                |
| $(\text{CH}_2)_3\text{CO}_2\text{H}$                      | $\text{CH}_3$                                | $\text{CO}_2\text{C}_2\text{H}_5$ | $\text{C}_1\text{H}_{11}\text{NO}_4\text{S}_2$                       | 122-123                                   | 71                |
| $(\text{CH}_2)_3\text{CO}_2\text{H}$                      | $\text{CH}_3$                                | $\text{CO}_2\text{H}$             | $\text{C}_7\text{H}_7\text{NO}_4\text{S}_2$                          | 203                                       | 89                |
| $(\text{CH}_2)_3\text{CO}_2\text{H}$                      | $\text{CH}_3$                                | H                                 | $\text{C}_{10}\text{H}_{15}\text{NO}_4\text{S}_2$                    | 86-87                                     | 70                |
| $\text{CHCO}_2\text{H}$                                   |                                              |                                   |                                                                      |                                           |                   |
| $\text{CH}_2\text{CO}_2\text{H}$                          | $\text{CH}_3$                                | H                                 | $\text{C}_8\text{H}_9\text{NO}_4\text{S}_2$                          | 217-218                                   | 26                |
| $\text{CH}_2\text{CH}_2\text{SO}_3\text{K}$               | $\text{CH}_3$                                | H                                 | $\text{C}_8\text{H}_9\text{NO}_4\text{S}_2\text{K}$                  | <sup>c</sup> 362                          | 20                |
| $\text{CH}_2\text{S}(\text{CH}_2)_2\text{CHCO}_2\text{H}$ | $\text{CH}_3$                                | H                                 | $\text{C}_{11}\text{H}_{13}\text{NO}_4\text{S}_2$                    | 130                                       | 80                |
| $\text{C}_6\text{H}_4\text{CO}_2\text{H-m}$               | $\text{CH}_3$                                | H                                 | $\text{C}_{11}\text{H}_9\text{NO}_4\text{S}_2$                       | <sup>b</sup> 191-193                      | 66                |

<sup>a</sup> Recrystallized from water unless otherwise indicated.

<sup>b</sup> From 50% ethanol.

<sup>c</sup> From methanol.

Preparation of a photosensitive composition according to the invention can be done by preparing an aqueous solution containing the photoactive silver complex simply by dissolving a water-soluble silver salt in aqueous solution with a near equimolar amount of a 3-substituted-4-thiazoline-2-thione selected from the class described above. Molar proportions of the silver salt and the 4-thiazoline-2-thione compound preferably should be kept about 1:1 in the solution although some variation from this ratio usually will be tolerable without seriously reducing photoactivity of the composition.

The silver complex can be mixed with gelatin or with other hydrophilic colloids such as polyvinyl alcohol, synthetic gelatin substitutes and the like, or a mixture thereof, to make a photographic emulsion for coating on a photographic support such as film, plates, paper or the like.

Following are specific examples describing in detail our most preferred mode for carrying out the invention.

#### EXAMPLE 1

Three separate solution parts are prepared.

Part A: To 20 milliliters distilled water add 0.62 gram of 3-(1-dicarboxyethyl)-4-methyl-4-thiazoline-2-thione and heat until a clear solution is obtained.

Part B: Dissolve 0.65 gram of p-toluenesulfonic acid, silver salt in 20 milliliters distilled water.

Part C: 40 Milliliters of 10 percent gelatin solution.

Pour Parts A and B simultaneously and slowly with continuous stirring into Part C. Add a few drops of saponin, filter the solution and then coat on conventional photographic paper support using a coating block with a coating knife set at 0.006 inch. After the coating has dried, the coated sample is exposed photographically on an Eastman 1B sensitometer through a step tablet for 30 seconds at positive film setting. The exposed sample is developed for 30 seconds at 75° F. in Kodak Developer D-76 diluted 1:1 with water then put through a

stop bath and washed thoroughly with water to remove undeveloped silver. Fixing by silver halide solvent is not necessary.

ry. A stepped silver image with low minimum density is obtained.

#### EXAMPLE 2

45 A sensitive emulsion is prepared and coated as in example 1 except using 0.68 gram of 3-(1-carboxyethyl)-4-methyl-4-thiazoline-2-thione and 0.9 gram p-toluenesulfonic acid silver salt instead of the corresponding quantities and components described in example 1. A photographic element is coated 50 with the emulsion as in example 1 and tested by the same procedure described in example 1 to produce a stepped silver image of good contrast and density.

55 Emulsions similar to those described in the above examples are prepared but using other 4-thiazoline-2-thiones that do have the acidic hydrogen-containing radical at the 3-position. None are found that have any significant photosensitivity. Similar emulsions made with the other 3-substituted-4-thiazoline-2-thiones named in the numbered list above and with those others described in table I are found to be 60 photosensitive to varying extents but all comparable with the preferred examples above.

The reaction between the soluble silver salt and the 4-thiazoline-2-thione is thought to be formation of a complex ion involving interaction of the silver ion and the active radical at the 3-position of the 4-thiazoline-2-thione, resulting in the silver salt complex. We have not yet definitely established the exact nature of the complex that is formed.

In the foregoing examples, we have described in detail only 70 some preferred embodiments of the invention for the purpose of setting out our most preferred mode of carrying out the invention. Other embodiments can involve variations from the specific examples described. Other compounds of the formula described above can be substituted for the specific 4-thiazoline-2-thione compounds used in the examples. The invention permits considerable variation in the methods that can

be used for preparing the light-sensitive coatings. Other components such as other soluble silver salts instead of the toluene-sulfonic acid silver salt, can be used or hydrophilic colloids other than gelatin can be substituted.

In defining the above formula, we have mentioned that there must be attached at the 3-position on the ring a group which contains an active hydrogen atom. This is necessary for photosensitivity of the silver complex. Also, it is necessary to photosensitivity that the thione sulfur atom must not be converted to a mercapto form. Compounds having acid groups at  $R_2$  or  $R_3$  positions can be used but, again, they are effective only if the  $R_1$  radical has the necessary active hydrogen atom. Compounds in table I are specific examples of compounds which the defined formula, useful for the invention.

In defining the above formula, we have mentioned that each of  $R_2$  and  $R_3$  can represent hydrogen or an organic radical. In table I we have described several preferred ones of such organic substituents, but these positions have not seemed critical to the photosensitive complex formation and we would include within our invention any 4-thiazoline-2-thione compound having the critical structure as defined and that forms a photosensitive complex with silver as described, regardless, of the nature of the  $R_2$  and  $R_3$  organic radical substituents.

With the foregoing statement in mind, we can mention that the  $R_2$  and  $R_3$  substituents in the formula can preferably include hydrogen, lower aliphatic radicals containing one to 10 carbon atoms, including radicals of lower aliphatic hydrocarbons, acids, esters, salts, ketones and the like, or can include aryl radicals, mixed aryl-alkyl radicals and the like. Substituents at these positions can affect solubility of the photosensitive complex and in preferred embodiments, the complexing agents can be selected for their better solubility characteristics, but our invention includes all embodiments that form the photosensitive complex.

Typical aliphatic groups having a terminal acidic hydrogen atom, which can constitute the  $R_1$  substituent, can include carboxyaliphatic, carboxythiaaliphatic and dicarboxyaliphatic, particularly carboxyalkyl and dicarboxyalkyl and including carboxythiaalkyl; sulfoaliphatic and hydroxy aliphatic such as sulfoalkyl and hydroxyalkyl. In most such groups comprising alkyl or thiaalkyl groups, the alkyl will preferably be alkyl containing one to six carbon atoms.

Photosensitive elements comprising the silver salt complexes of the invention as essential photosensitive components can be in a variety of forms. The elements can comprise any suitable support. Typical supports can be paper or film sheets, glass or metal plates and the like, for example, baryta coated or plain paper supports or papers coated with a resin coat such as polyethylene or other polyolefin. The support can be a film support such as cellulose esters or polyester films, particularly the cellulose acetates or polyethylene terephthalate films. The elements can comprise one, or more than one, photosensitive-recording layer and in multiple layer elements the elements can comprise photosensitive layers of other compositions in combination with a separate recording layer of a silver salt complex described herein. Elements comprising one or more recording layers of the silver salt complexes can be made for various uses such as color photography, X-ray recording, ultraviolet recording and the like. The recording layer comprising the silver salt complex can be coated without a binder for some applications or can be coated in a layer comprising any suitable binder, including particularly hydrophilic colloids such as gelatin, polyvinyl alcohol and other synthetic polymer hydrophilic colloids. The silver salt complexes can be sensitized to improve photographic speed with chemical sensitizers and can be sensitized with spectral sensitizing dyes. Generally, chemical and spectral sensitizers known for use in silver halide photographic emulsions can be included in recording layers containing the silver salt complexes of this invention. Layers comprising the silver salt complexes can be the photosensitive layer or a diffusion transfer photographic element, and in some embodiments can be used in diffusion transfer processes without need for a specific silver salt solvent, as many of the silver salt complexes will be soluble

enough in the developer solution without need for a specific solvent. The silver salt complexes can be developed known for use with silver halides, employing the conventional developing agents. When desired, a physical developer may be employed to intensify the developed silver image.

The silver salt complexes are useful as the photosensitive silver salt in a dry development system in which an image is developed by a dry physical development process. An incorporated silver salt such as silver behenate, in presence of a reducing agent is capable of intensifying the image by a dry heat process. A process of this kind, but using different photosensitive silver salts, is described in U.S. Pat. No. 3,152,904 patented Oct. 13, 1964 to David P. Sorensen et al.

Photosensitive emulsions comprising the silver salt complexes can be coated by conventional coating techniques that are employed for coating silver halide emulsions. The emulsions can contain adjuvants employed in various silver halide emulsions such as conventional wetting agents, hardeners, antifoggants, dyes, dye precursors in color imaging layers, and the like.

Although the invention has been described in detail with particular reference to preferred embodiments thereof, variations and modifications can be effected within the spirit and scope of the invention as described hereinbefore and as defined in the appended claims.

We claim:

1. A photographic element comprising a support and coated thereon a photosensitive recording layer comprising, as an essential photosensitive component thereof, a silver salt complex of a 3-substituted-4-thiazoline-2-thione compound having the formula:



40 wherein  $R_1$  is an aliphatic radical containing from one to 12 carbon atoms which has a terminal acidic hydrogen atom bonded to an oxygen atom and salts thereof, and  $R_2$  and  $R_3$  respectively are each selected from the group consisting of hydrogen, aliphatic radicals or a phenyl radical.

45 2. A photographic recording element defined by claim 1 wherein  $R_1$  is a carboxy aliphatic radical.

3. A photographic recording element defined by claim 1 wherein  $R_1$  is a carboxy alkyl radical.

4. A photographic recording element defined by claim 1 wherein  $R_1$  is carboxymethyl.

5. A photographic recording element defined by claim 1 wherein  $R_1$  is carboxyethyl.

6. A photographic recording element defined by claim 1 wherein  $R_1$  is a dicarboxyaliphatic radical.

55 7. A photographic recording element defined by claim 1 wherein  $R_1$  is a dicarboxyalkyl radical.

8. A photographic recording element defined by claim 1 wherein  $R_1$  is dicarboxyethyl.

9. A photographic recording element defined by claim 1 wherein  $R_1$  is a sulfoaliphatic radical.

60 10. A photographic recording element defined by claim 1 wherein  $R_1$  is a sulfoalkyl radical.

11. A photographic recording element defined by claim 1 wherein  $R_1$  is sulfoethyl.

65 12. A photographic recording element defined by claim 1 wherein  $R_1$  is a carboxy thia-aliphatic radical.

13. A photographic recording element defined by claim 1 wherein  $R_1$  is a carboxy thia-alkyl radical.

14. A photographic recording element defined by claim 1 wherein  $R_1$  is carboxythiapentane.

70 15. A photographic recording element defined by claim 1 wherein  $R_1$  is a hydroxyaliphatic radical.

16. A photographic recording element defined by claim 1 wherein  $R_1$  is a hydroxyalkyl radical.

75 17. A photographic recording element defined by claim 1 wherein  $R_1$  is hydroxyethyl.

18. A photographic recording element defined by claim 1 wherein R<sub>2</sub> and R<sub>3</sub> can each be hydrogen atoms, aliphatic radicals containing from one to 10 carbon atoms or phenyl.

19. A photographic emulsion comprising a silver salt complex of a 3-substituted-H-thiazoline-2-thione having the formula:



wherein R<sub>1</sub> is an aliphatic radical containing from one to 12 carbon atoms which has a terminal acidic hydrogen atom bonded to an oxygen atom and salts thereof, and R<sub>2</sub> and R<sub>3</sub>

respectively are each selected from the group consisting of hydrogen, aliphatic radicals or a phenyl radical, as an essential photosensitive component of said emulsion.

20. A photographic emulsion according to claim 19, wherein R<sub>1</sub> is a carboxy aliphatic radical and R<sub>2</sub> and R<sub>3</sub> are each hydrogen atoms, lower aliphatic radicals containing one to 10 carbon atoms or phenyl.

21. A photographic emulsion comprising a silver salt complex of 3-(1,2-dicarboxyethyl)-4-methyl-4-thiazoline-2-thione as an essential photosensitive component of said emulsion.

22. A photographic emulsion comprising a silver salt complex of 3-(1-carboxyethyl)-4-methyl-4-thiazoline-2-thione as an essential photosensitive component of said emulsion.

23. A photographic emulsion according to claim 19 wherein the aliphatic radical is a lower alkyl radical, an acid radical or salt thereof, an ester radical, a ketone radical, or an aryl or a mixed aryl-alkyl radical.

\* \* \* \* \*

UNITED STATES PATENT OFFICE  
CERTIFICATE OF CORRECTION

Patent No. 3,620,749 Dated November 16, 1971

Inventor(s) Grant M. Haist, Wilbert J. Humplett, James R. King

It is certified that error appears in the above-identified patent and that said Letters Patent are hereby corrected as shown below:

Col. 1, line 17, "photography" should read ---photograph---.

Col. 1, line 55, "4-carbosy" should read --- 4-carboxy ---.

Col. 2, line 9, "3-substituted-4-thiazoline-2thiones" should read --- 3-substituted-4-thiazoline-2-thiones ---.

Col. 2, line 11, "6aminohexanoic" should read --- 6-aminohexanoic

Col. 2, line 19, "4Acetoxyethyl-3-(2carboxyethyl)" should read --- 4-Acetoxyethyl-3-(2-carboxyethyl) ---.

Col. 2, line 42, "3-(2carboxyethyl)" should read --- 3-(2-carboxyethyl) ---.

Col. 3, line 1, "-2thiones" should read --- -2-thiones ---.

Col. 3, line 62, "(1,-dicarboxyethyl)" should read --- (1,2-dicarboxyethyl) ---.

Col. 5, line 14, "which the defined formula," should read ---within the defined formula---.

Claim 19, line 2, "3-substituted-H-thiazoline" should read --- 3-substituted-4-thiazoline ---.

Signed and sealed this 2nd day of January 1973.

(SEAL)  
Attest:

EDWARD M.FLETCHER,JR.  
Attesting Officer

ROBERT GOTTSCHALK  
Commissioner of Patents